

Jan. 27, 1970

F. TROMBE ET AL

3,492,084

PROCESS FOR SEPARATING RARE EARTHS

Filed Aug. 29, 1966

2 Sheets-Sheet 1

*Fig. 1.*



*Fig. 2.*



Jan. 27, 1970

F. TROMBE ET AL

3,492,084

PROCESS FOR SEPARATING RARE EARTHS

Filed Aug. 29, 1966

2 Sheets-Sheet 2



## 1

3,492,084

PROCESS FOR SEPARATING RARE EARTHS  
Félix Trombe, Paris, France, and Paul Caro, Tempe,  
Ariz., assignors to Centre National de la Recherche  
Scientifique, Paris, France

Filed Aug. 29, 1966, Ser. No. 575,847

Claims priority, application France, Oct. 11, 1965,

34,522

Int. Cl. C22b 59/00

U.S. Cl. 23—15

5 Claims

## ABSTRACT OF THE DISCLOSURE

A mixture of rare earths is separated into a fraction containing rare earths whose carbonates are relatively more soluble and a fraction of rare earths whose carbonates are relatively less soluble, by contacting a mixture of rare earth carbonates and soluble rare earth salts in the presence of carbon dioxide.

The invention pertains to a process for separating a mixture of rare earths (in which will be included elements such as yttrium and scandium) into its individual components.

According to the process of the invention, one reacts a suspension consisting of a mixture of carbonates of the rare earth elements to separate them from one another, in the presence of carbon dioxide, with an aqueous solution of soluble salts of the same rare earth elements.

This aqueous solution may have initially the same rare earth element composition as said suspension.

It has been found, on the one hand, that the solubilities in an aqueous solvent of most of the different rare earth elements, though remaining very low, increases together with the concentration of carbon dioxide in the aqueous solvent and that, on the other hand, the differences in the solubilities with respect to one another of the respective rare earth elements increase as a function of the concentration of carbon dioxide dissolved in the aqueous medium. Broadly speaking, the solubilities of the respective rare earth elements considered increase with their atomic numbers in the presence of dissolved carbon dioxide in the aqueous solvent, the lightest, such as lanthanum and cerium being the most insoluble and the heaviest, such as erbium, being the most soluble. The solubility of the yttrium carbonate is intermediate between those of the carbonates of the rare earths neodymium and erbium while scandium carbonate finds its place among the most soluble carbonates of the heaviest rare earths.

These phenomena are illustrated by the curves of FIGURE 1 which show the variations of the solubilities of the carbonates of the rare earth elements in water, at 22° C., in function of the pressure of carbon dioxide in contact with the solution.

The measurements were made in a vessel, starting from pure rare earth carbonates suspended in water (2 or 3 grams per litre), by subjecting them to the action of carbon dioxide (in pure form or diluted with argon) for 4–5 hours at a predetermined temperature, in the present instance at 22° C., under increasing pressures of CO<sub>2</sub>.

The solution recovered in each experience was treated with HCl, heated to boiling to completely remove CO<sub>2</sub>. The dissolved rare earth salt was then precipitated in the form of the hydroxide with ammonia and calcined into oxides which were then weighed.

FIGURE 1 shows clearly the increase in the solubility (plotted on the ordinate and expressed in mg. per litre of the corresponding oxides) of most of the rare earth carbonates (as a function of the absolute pressure of carbon dioxide plotted on the abscissa in mm. of mercury) and further shows the increasing differences in the

## 2

solubilities with respect to one another of the different carbonates as a function in the increase of the pressure of carbon dioxide above the aqueous solution.

It has been noted that, when the CO<sub>2</sub> pressure is increased beyond one atmosphere, the solubilities of the different carbonates remain quite unchanged, except for the carbonates of the heaviest rare earth elements such as erbium (and scandium) the solubilities of which keep increasing slightly when the carbon dioxide pressure is increased up to 3 atmospheres.

It has been further found that the solubilities of the rare earth carbonates in the presence of a determined pressure of carbon dioxide increase as the temperature decreases. The lower the temperature, the higher the solubility of the rare earth carbonates.

FIGURES 2 and 3 show respectively the variations of the solubilities of the yttrium carbonate and scandium carbonate respectively as a function of the temperature in the presence of carbon dioxide under pressures of 250, 20 380, 502 and 760 mm. of mercury.

However, these solubilities remain in any case so low that the separation of rare earths by a simple selective dissolution of a mixture of their carbonates in water may not be carried out on an industrial scale as is evidenced by the experiences described herebelow which, nevertheless, show the important modifications of the composition of solubilized rare earths fraction as compared with the starting composition of the mixture.

The starting product consisted of a mixture of rare earth hydroxides having the composition shown in the middle column of Table I herebelow. Four batches, each of which consisted of five kilograms of hydroxides (containing about 70% of rare earth oxides), were treated with carbon dioxide which was allowed to bubble into the suspension, this treatment being repeated several times for removing soluble impurities and the calcium. The bubbling of CO<sub>2</sub> was continuously maintained under a pressure of 3 atmospheres in order to avoid hydrolysis back to the hydroxides of the carbonates obtained.

More specifically, these batches were suspended under vigorous stirring in 150 l. of water within a stainless steel vessel filled with carbon dioxide under a pressure of 3 atmospheres. After a 24 hour contact between the suspension and the carbon dioxide, the solutions recovered in the 4 experiences contained from 17 to 24 gr. (per 150 l. of water) of rare earth and yttrium oxides, e.g. from 117 to 166 mg./l.

The composition of the rare earth mixture extracted from the liquid phase is shown in the right hand side column of Table I (the rare earths were dosed by X-fluorescence by means of the borax bead process).

TABLE I

| Elements | Composition after reaction                                                                                   |                                                                                                     |  |
|----------|--------------------------------------------------------------------------------------------------------------|-----------------------------------------------------------------------------------------------------|--|
|          | Proportions expressed in oxide weight percent of the respective rare earth elements in the carbonate mixture | Proportions expressed in oxide weight percent of the respective rare earth elements in the solution |  |
| Y        | 8                                                                                                            | 28                                                                                                  |  |
| Pr       | 7.5                                                                                                          | 3.5                                                                                                 |  |
| Nd       | 39.5                                                                                                         | 24.5                                                                                                |  |
| Sm       | 12.5                                                                                                         | 6.5                                                                                                 |  |
| Gd       | 10                                                                                                           | 9                                                                                                   |  |
| Dy       | 3.5                                                                                                          | 5                                                                                                   |  |
| La, Ce   | Not dosed                                                                                                    | Not dosed                                                                                           |  |

It will be noted that the solution is highly enriched in yttrium. This table thus confirms that there is a remarkable difference in solubilities between, for instance, the carbonate of neodymium and the carbonate of yttrium.

The yield of this enrichment operation is, however, extremely low and is of no practical use, due to the minor solubilities of the rare earth carbonates.

However, according to the process of the invention, advantage is taken of these differences in solubilities for separating the rare earth elements from a mixture thereof by reacting a suspension of the mixture of the rare earth elements in the form of their carbonates, in the presence of carbon dioxide, with an aqueous solution of soluble salts of the same elements, this solution containing, if the case should be, the same initial cationic proportions of said elements, whereby the solid phase suspended becomes more concentrated in those of the rare earths whose carbonates exhibit the smallest solubilities and the solution in the salts of the elements whose carbonates exhibit the greatest solubilities.

It will be noted that the process according to the invention takes advantage of the so-called metatactic reactions which are known for metallic hydroxides.

As a matter of fact, when a soluble salt  $XA$  of a cation  $X$  and an insoluble salt  $YB$  of a cation  $Y$ , are brought into contact, the cations  $X$  and  $Y$ , on the one hand, and the anions  $A$  and  $B$ , on the other hand, being selected such that the salt  $XB$  is much more insoluble than the salt  $YB$ , there occurs the following reaction:



which causes cation  $Y$  to go into solution.

Such a type of reaction is known in connection with the hydroxides of copper, zinc and cadmium which exhibit, respectively, the following solubility products:

|            |              |
|------------|--------------|
| $Cu(OH)_2$ | $10^{-19.7}$ |
| $Zn(OH)_2$ | $10^{-16.9}$ |
| $Cd(OH)_2$ | $10^{-14.2}$ |

The corresponding nitrates however are highly soluble in water.

The reaction of zinc hydroxide or cadmium hydroxide suspended in water with the soluble copper nitrate causes the complete dissolution of the zinc or cadmium in the form of their nitrates according to the following reaction:



In the practice of the process of the invention the raw material consisting of a mixture of hydroxides such as, for instance, the mixture considered in the previous selective dissolution example (see middle column of Table II), is first suspended in water and converted into carbonates in the presence of carbon dioxide and reacted with another portion of the above starting mixture which has been previously treated with a dosed solution of the hydrochloric acid to convert the rare earth into soluble chlorides.

Alternatively the process may also be carried out by first suspending the starting mixture of hydroxides in an aqueous medium and by adding thereto an amount of hydrochloric acid (or if the case should be of another acid the rare earth salts of which are soluble) dosed for dissolving only part of hydroxides mixture.

The suspension is then subjected to carbonation by bubbling carbonic dioxide through the suspension for a time sufficient to enable the metatactic reaction to take place.

It will be of course appreciated that the molar proportion of hydrochloric acid used with respect to the quantity of rare earth oxides treated will act on the final distribution conditions of the rare earth cations in the solid phase as well as in the solution.

In order to illustrate the foregoing, a non limitative example will be given hereafter for illustrating the process according to the invention.

The starting mixture consisted of 5 kg. of the hydroxides, mixture used already in the above disclosed examples and which, through calcination, yields 3.5 kg. of

oxides. These hydroxides were suspended in 150 l. of water under a vigorous stirring.

1.5 l. of an hydrochloric acid solution of 22-23° C. Baumé, e.g. 1.785 kg. of this solution containing 660 gr. of HCl, were added to the suspension and carbon dioxide was then bubbled into the suspension during 48 hours under a pressure of 3 atmospheres.

A solution of chlorides corresponding to an amount of 510 gr. of oxides whose composition is reported in the right hand side column of Table II, herebelow, is obtained:

TABLE II

| Elements | Composition after metatactic reaction                          |                                                               |
|----------|----------------------------------------------------------------|---------------------------------------------------------------|
|          | Composition in oxide weight percent of solid carbonate mixture | Composition expressed in oxide weight percent of the solution |
| Y        | 5                                                              | 27                                                            |
| Pr       | 9                                                              | 7                                                             |
| Nd       | 42                                                             | 26.5                                                          |
| 20 Sm    | 15.5                                                           | 7.5                                                           |
| Gd       | 10                                                             | 9.5                                                           |
| Dy       | 2                                                              | 4.7                                                           |
| Ce       | 8                                                              | 0                                                             |
| La       | 10                                                             | 11                                                            |

It will be noted that the proportions of yttrium and, as a general rule, of the other rare earths with respect to one another in the solution is about the same than the one obtained in the former example through simple selective dissolution of the starting hydroxides in the presence of carbon dioxide. However, the quantity of rare earths extracted from the same volume of the solution obtained, starting from the same mixture, passes from 24 gr. to 510 gr., thus to an extracted quantity which has been multiplied by a factor of about 20, such multiplication enabling the application of this process to industrial separations, the same steps being repeated either on the separated carbonate mixture or on the mixture recovered from the solution, for instance by reaction with ammonia to transform again the solubilized rare earth chlorides into the hydroxides.

By modifying the above example factors (such as a different proportion of HCl or a decrease of the temperature under which the process is operated at a temperature close to 0° C.) this multiplication factor may be highly increased up to a one hundred value. Other acids, such as  $HNO_3$ , may replace HCl.

This process is particularly effective for separating for instance a mixture of neodymium and yttrium. An example of this separation will be described in connection with FIGURE 4 which, diagrammatically, represents the variations of the compositions of the liquid phase (curve I) and of the solid phase (curve II) in equilibrium therewith, as a function of the composition of the starting mixture (whose varying compositions in yttrium and neodymium are represented by points on the represented diagonal line of the square diagram) when the starting mixture of neodymium and yttrium hydroxides, suspended in water, has been treated with the amount of hydrochloric acid which dissolves 20.8 percent of the starting mixture and has further been subjected to the carbon dioxide bubbling until completion of the reaction.

For instance, assuming that the starting mixture contains 30% of neodymium and 70% of yttrium (the composition of this mixture being represented by point *a* on the diagonal line of the square diagram), the final compositions of the liquid phase and solid phase will respectively be represented by points *c* and *b* (which compositions are read on the ordinate) at the intersection of a line parallel to the ordinate passing by *a* with the two curves I and II.

It will be appreciated that the solid phase became richer in the element whose carbonate is the less soluble (it contains about 55% of neodymium and 45% of yttrium) whereas the solution became richer in yttrium whose carbonate is the more soluble (it contains about 20% of neodymium and 80% of yttrium).

The extraction operation may be repeated either on the solid phase (whose starting composition is represented by  $c_1$  on the diagonal line) or on the mixture of hydroxides precipitated, for instance with ammonia, from the liquid phase (whose starting composition is represented by  $b_1$  on the diagonal line).

In the first instance a more highly neodymium enriched precipitate exhibiting the composition  $e$  is obtained in equilibrium with a solution whose composition is represented at  $d$ .

In the second instance a more highly enriched yttrium solution exhibiting the composition  $f$  is obtained in equilibrium with a solid phase whose composition is represented at  $d$ .

It will be readily appreciated that, by repeating these operations a few times on the precipitates obtained in the first instance and on the solution obtained in the second instance, a pure solid neodymium carbonate phase and a pure yttrium chloride solution respectively will be obtained rapidly.

In some instances, the separation may be perfected, in a final step, by passing solutions of the soluble chlorides of the purified rare earth fraction through a column of ion exchange resin as is well known in the art.

There is thus provided a new process enabling an efficient separation at low cost and by using the most conventional reaction materials.

What we claim is:

1. A process of separating a mixture of rare earths into a first fraction enriched with respect to rare earths whose carbonates are more soluble and a second fraction enriched with respect to rare earths whose carbonates are less soluble comprising the steps of contacting a suspension comprising a plurality of rare earth carbonates, in the presence of carbon dioxide, with a solution comprising a plurality of soluble rare earth salts, at least some of the rare earths elements of said soluble salts and of said carbonates being the same, to provide a liquid phase containing soluble rare earth salts enriched with respect to rare earths whose carbonates are more soluble and a solid

phase enriched in rare earths whose carbonates are less soluble, said carbon dioxide being present in an amount sufficient to permit a substantial separation of said rare earths.

5 2. A process according to claim 1, wherein said solution contains said rare earth soluble salts in the same proportions with respect to one another as in said mixture of carbonates.

3. A process according to claim 1, wherein said rare earth soluble salts consists of rare earth chlorides.

10 4. A process of separating a mixture of rare earths into a first fraction enriched with respect to rare earths whose carbonates are more soluble and a second fraction enriched with respect to rare earths whose carbonates are less soluble comprising the steps of providing a suspension of a plurality of rare earth hydroxides in water, treating said suspension with an inorganic acid to convert a portion only of said rare earth hydroxides into soluble rare earth acid salts, and contacting the resulting reaction mixture with carbon dioxide to provide a solid phase enriched in respect to rare earths whose carbonates are less soluble and a liquid phase enriched in respect to rare earths whose carbonates are more soluble, said carbon dioxide being present in an amount sufficient to permit a substantial separation of said rare earths.

20 5. A process according to claim 4 wherein said inorganic acid comprises hydrochloric acid.

#### References Cited

##### UNITED STATES PATENTS

|           |         |                 |       |         |
|-----------|---------|-----------------|-------|---------|
| 2,872,287 | 2/1959  | Duffield et al. | ----- | 23—22 X |
| 3,092,449 | 6/1963  | Bril et al.     | ----- | 23—23 X |
| 3,153,571 | 10/1964 | Bronaugh        | ----- | 23—61 X |
| 3,401,008 | 10/1968 | Head            | ----- | 23—23   |

35 HERBERT T. CARTER, Primary Examiner

40 U.S. Cl. X.R.

23—18, 19, 20, 23, 61, 87, 102, 183